

## UNITED STATES PATENT OFFICE.

ROBERT G. GUTHRIE AND OSCAR J. WOZASEK, OF CHICAGO, ILLINOIS, ASSIGNORS TO  
PEOPLES GAS BY-PRODUCTS CORPORATION, OF CHICAGO, ILLINOIS, A CORPORA-  
TION OF ILLINOIS.

## PROCESS OF CARBURIZING IRON AND STEEL.

No Drawing.

Application filed January 2, 1929. Serial No. 329,942.

The invention relates to new and useful improvements in a process of carburizing iron or steel by a gaseous treatment. (The present application is a continuation in part 5 of our prior application Serial No. 220,632, filed September 19, 1927.)

An object of the invention is to produce a carburized steel of given depth of case in less time than has been required by former processes.

A further object of the invention is to provide a process wherein the carburizing efficiency of a carbonaceous gas is increased.

A still further object of the invention is to provide a process wherein the carbon concentration of the case is increased for a given depth of penetration.

A still further object of the invention is to provide a process wherein the acceptability 20 of the iron or steel is increased for a given carbonaceous gas.

These and other objects will in part be obvious and will in part be hereinafter more fully disclosed.

25 The invention in its broadest aspect relates to a process of carburizing iron or steel which consists in heating the iron or steel to an elevated temperature in a container or retort and subjecting said iron or steel while 30 maintained at the elevated temperature to a carbonaceous matter, preferably a carbonaceous gas. The carbonaceous gas may be of any well known character, but to get the best efficiency must be a practically dry or dehydrated carburizing gas. It is found in practice that "city gas" being the illuminating 35 gas delivered through mains in cities, is excellently adapted for the purpose. This gas is often referred to as "town gas."

40 The process also includes the introduction into the retort while at an elevated temperature of a minute quantity of oxygen, either free or combined. The oxygen is introduced either immediately before or simultaneously 45 with the initial introduction of the carbonaceous gas. It is essential that the oxygen shall be introduced at this beginning of the treatment with the carbonaceous gas so as to form an oxide catalyst, which greatly increases 50 the rapidity of penetration of the carbon into the iron or steel during the subjecting of the iron or steel to the action of the carbonaceous gas. By this increasing of the

rapidity of the penetration the period of time necessary to obtain a given depth of case with 55 a given gas is materially decreased.

When certain reluctant steels and irons, such as the so-called "abnormal steels and irons" are to be treated, sulphur, either free or combined, is added in minute quantities 60 to the retort. When sulphur is added, a greater concentration of carbon for a given depth of case is obtained in a given time. The addition of the sulphur increases the acceptability for carbon of the so-called "abnormal iron or steel." Sulphur may be added 65 to the retort at the beginning of the treatment with the carbonaceous gas. Excellent results have been obtained, however, by adding the sulphur in minute quantities at other times during the carburizing process and continuously throughout the carburizing process.

In order to aid in an understanding of the process we will describe more in detail one 75 manner in which the process has been carried out. A 1500-pound vertical cylindrical retort type of carburizing furnace was used. This was filled with the steel and iron parts to be carburized and the entire mass was 80 brought to a temperature between 1500 and 1800 degrees F. When the temperature reached approximately 1750 degrees F., the "town gas" was allowed to enter the bottom 85 of the retort and coincidental with the introduction of the gas, ten drops of water permitted for a total of three minutes was allowed to drip into the inflowing gas. This supplied the oxygen to form the oxide catalyst. In the carrying out of this process, the 90 carbonaceous gas was supplied continuously throughout the run and for the first three minutes only of the run oxygen was added in the manner stated, after which the supply of the water was cut off and the supply of the 95 carbonaceous gas continued. The carbonaceous gas passed over the iron and steel parts and out of an exit at the top where it was burned to prevent contamination of the atmosphere.

100 It was found by this process that the rapidity of penetration of the carbon into the iron and steel during the carburizing of the same was greatly increased in order to obtain a given depth of case. This was accomplished by increasing the carburizing effi- 105

ciency of the carbonaceous gas by the action of the oxide catalyst formed at the beginning of the run.

The sulphur which is used in connection with certain irons and steels may be introduced in minute quantities by adding sulphur dioxide to the carbonaceous gas in which case, if added at the beginning of the run, the sulphur dioxide will supply sufficient oxygen to form the oxide catalyst. It will be understood, however, that the sulphur may be introduced into the retort in various ways. It will also be understood that the oxygen may be supplied to the retort in other forms. It is essential, however, in connection with the oxygen that a very minute quantity shall be introduced into the retort at the beginning of the run, and in connection with the sulphur, a minute quantity is introduced into the retort either at the beginning of the run or at any time during the treatment of the iron and steel with the carbonaceous gas. With the use of sulphur it is possible to carburize and at the same time reduce or minimize the abnormality of an abnormal iron or steel in the presence of a carbonaceous gas of normally low carburizing efficiency. In other words, by this process the oxygen iron catalyst increases the efficiency of the inherent efficient carbonaceous gas and the sulphur increases the acceptability for carbon of the so-called "abnormal iron or steel".

It will be understood that the invention may be carried out in other ways without departing from the spirit thereof as set forth in the appended claims.

Having fully described our invention, what we claim as new and desire to secure by Letters Patent, is:—

1. The process of carburizing iron or steel comprising heating the iron or steel to an ele-

vated temperature in a container or retort, subjecting said iron or steel while maintained at the elevated temperature to a carbonaceous gas and treating said iron or steel at the beginning of the treatment with the carbonaceous gas with a minute quantity of oxygen to form an oxide catalyst whereby the rapidity of penetration of the carbon into the iron or steel during the carburizing of the same is 45 greatly increased.

2. The process of carburizing iron or steel comprising heating the iron or steel to an elevated temperature in a container or retort, subjecting said iron or steel while maintained at the elevated temperature to a dehydrated carbonaceous gas and treating said iron or steel at the beginning of the treatment with the carbonaceous gas with a minute quantity of oxygen to form an oxide catalyst 55 whereby the rapidity of penetration of the carbon into the iron or steel during the carburizing of the same is greatly increased.

3. The process of carburizing iron or steel comprising heating the iron or steel to an 60 elevated temperature in a container or retort, subjecting said iron or steel while maintained at the elevated temperature to a carbonaceous gas, treating said iron or steel at the beginning of the treatment with the carbonaceous gas with a minute quantity of oxygen to form an oxide catalyst and with a minute quantity of sulphur during the treatment with the carbonaceous gas whereby the 65 efficiency of the carbonaceous gas is increased and the acceptability of the iron or steel for carbon is increased.

In testimony whereof, we affix our signatures.

ROBERT G. GUTHRIE.  
OSCAR J. WOZASEK.